

## UNITED STATES PATENT OFFICE

1,945,371

METHOD OF TREATING COAL AND  
PRODUCT THEREOF

Nathaniel R. Landon, Mount Kisco, and Ernest  
Victor Collins, Jr., Brooklyn, N. Y., assignors  
to Delaware, Lackawanna & Western Coal  
Company, New York, N. Y., a corporation of  
New Jersey

No Drawing. Application February 14, 1930  
Serial No. 428,511

## 7 Claims. (Cl. 44—6)

This invention relates to the treatment of coal that has become discolored either in storage or below the surface to restore essentially the original appearance of bright black coal.

5 The consuming public, who are accustomed to recognize anthracite coal by its jet black color and luster often assume that coal which is dull or discolored and has thus lost its characteristic appearance is poor in quality. Coal that has 10 become discolored cannot be restored to its original jet black appearance by ordinary washing. Consequently serious losses are sustained by the producer because this dull or discolored coal does not command the price of coal that is black and 15 bright in appearance although analysis indicates that the change is only one of appearance and there is no loss of fuel value or consequential change in chemical composition.

It is the object of the present invention to provide 20 a practical method of treating discolored coal to restore its original characteristic appearance.

The iron in the mineral matter of coal is considered to be almost wholly present in combination 25 with sulphur. Under the influence of atmospheric exposure or subjected to mildly acid mine water, the iron sulphides become oxidized presumably to insoluble basic sulphates, oxides and other compounds imparting to the coal a rusty 30 appearance. Other reactions go on and other metallic compounds may show on the surface. This is particularly true of storage coal and consequently the longer it is exposed to atmospheric influences or acid water, the greater becomes the 35 discoloration.

We have discovered that the original appearance 40 of discolored coal can be restored by treating the coal under appropriate conditions with tanning materials in general. The term "tanning materials" as here used includes a variety of reagents which combine with iron compounds and when oxidized produce bleach compounds on the 45 surface of the coal. Among such reagents are tannin or tannic acid, gallic acid, pyrogallic acid or pyrogallol and extracts such as quebracho, chestnut, cutch, divi-divi, gambier, myrobolans, nutgalls, sumac, valonia, hemlock, spruce, oak-bark, wattle and the like. We have also discovered 50 that extract of logwood may be applied advantageously to discolored coal either alone or in combination with one or more of the tanning materials mentioned.

As an example of the method we may proceed as follows: a 5% solution by weight of gallic or pyrogallic acid is heated, preferably to ap-

proximately 180° F. The discolored coal is immersed in this solution for a period sufficient to accomplish the object, usually about one minute, after which the coal is removed on a slow conveyor in which the coal is exposed to the atmosphere so that the solution dries on the coal and the iron compounds formed with the reagent used are oxidized. We have found that the best results are secured if the solution is maintained in a slightly alkaline condition. A suitable alkali such as sodium carbonate can be added in proportions to maintain the acid condition.

As another example we may employ a 20% solution by weight of sumac at approximately 180° F. The coal is introduced to a tank containing this solution and is permitted to remain therein for about 45 seconds. It is withdrawn by a conveyor moving at a slow rate to permit drying and oxidation.

We prefer to immerse the coal in the solution, 75 but the solution can be sprayed or applied otherwise to the coal, so long as the discolored coating is saturated with the reagent. The excess solution which is drained from the coal can be returned and reused.

As hereinbefore indicated, we may employ similarly an extract of logwood in solution with or without the addition of one or more of the reagents mentioned.

Coal which has been treated as hereinbefore 85 described presents the characteristic appearance of freshly mined coal. The losses heretofore incident to the storage of coal and consequent discoloration thereof are avoided by the application of the simple and effective procedure described. 90

The term "tannins" as used in the accompanying 95 claims includes the reagents hereinbefore mentioned and their equivalents. Equivalent reagents are such as may react with iron compounds on the surface of the coal to produce a black coating.

Various changes may be made in the details of operation and in the reagents employed without departing from the invention or sacrificing 100 any of the advantages thereof.

We claim:

1. The method of treating coal which is discolored by oxidized iron compounds which comprises subjecting the coal to the action of a tannin solution and exposing the coal thereafter to the atmosphere whereby the oxidized iron compounds are converted into other compounds which restore the natural appearance of the coal.
2. The method of treating coal which is dis-

- colored by oxidized iron compounds which comprises subjecting the coal to a solution containing a reagent of the group consisting of tannic acid, gallic acid and pyrogallic acid and exposing the coal thereafter to the atmosphere whereby the oxidized iron compounds are converted into other compounds which restore the natural appearance of the coal.
3. The method of treating coal which is discolored by oxidized iron compounds which comprises subjecting the coal to a solution of an extract containing a reagent of the group consisting of tannic acid, gallic acid and pyrogallic acid, and exposing the coal thereafter to the atmosphere whereby the oxidized iron compounds are converted into other compounds which restore the natural appearance of the coal.
4. The method of treating coal which is discolored by oxidized iron compounds which comprises subjecting the coal to the action of an alkaline solution containing a tannin and exposing the coal thereafter to the atmosphere whereby the oxidized iron compounds are converted into other compounds which restore the natural appearance of the coal.
5. The method of treating coal which is discolored by oxidized iron compounds to restore the natural appearance thereof which comprises converting the iron compounds into black compounds by reaction with a tannin. 80
6. The method of treating coal which is discolored by oxidized iron compounds which comprises treating the coal with an extract of logwood and exposing the coal thereafter to the atmosphere whereby the oxidized iron compounds are converted into other compounds which restore the natural appearance of the coal. 85
7. The method of treating coal which is discolored by oxidized iron compounds which comprises treating the coal with an extract of logwood and a tannin and exposing the coal thereafter to the atmosphere whereby the oxidized iron compounds are converted into other compounds which restore the natural appearance of the coal. 90
- NATHANIEL R. LANDON.  
ERNEST VICTOR COLLINS, JR. 95
- 100
- 105
- 110
- 115
- 120
- 125
- 130
- 135
- 140
- 145
- 150